# EUROPEAN PATENT SPECIFICATION

(11) **EP 0 686 182 B1**
(45) Date of publication and mention of the grant of the patent: **03.11.1999**
(21) Application number: 94909061.7
(22) Date of filing: 24.02.1994
(51) Int. Cl.: C10L 1/22, C10L 1/28, C10L 1/02

(54) **OIL ADDITIVES AND COMPOSITIONS**
ÖLEZUSÄTZE UND ZUSAMMENSETZUNGEN
COMPOSITIONS A BASE DE PETROLE ET ADJUVANTS POUR PETROLE

(30) Priority: 26.02.1993 GB 9303924
(43) Date of publication of application: 13.12.1995
(73) Proprietor: Infineum USA L.P., Linden, New Jersey 07036 (US)
(72) Inventor: DAVIES, Brian, William, Blewbury Oxfordshire OX11 9PD (GB); LOMBARDI, Alessandro, Abingdon Oxfordshire OX13 5QF (GB)
(74) Representative: Bawden, Peter Charles
(86) International application number: EP9400550
(87) International publication number: WO9419430

(56) References cited:
- WO-A-94/06894
- FR-A- 1 584 938
- FR-A- 2 579 481
- GB-A- 658 494
- US-A- 2 862 885
- US-A- 4 364 743
- US-A- 5 192 336

## Description

This invention relates to oil compositions, primarily to fuel oil compositions, and more especially to the control of foaming in such compositions.

In the processing and transport of hydrocarbon oils, foaming frequently occurs as the oil is passed from one vessel to another. The foaming may interfere with the pumping of the oil, and may be such as to require a reduction in pumping rate to allow foam collapse to avoid oil spills. It is desirable to control foaming to permit higher rates of oil transfer.

The problem of foaming is particularly important in the distribution of oils such as liquid petroleum oils, especially fuel and lubricant oils. Such oils typically pass through a distribution network, involving pumping through pipelines, or a series of storage tanks.

Fuel oils derived from vegetable or animal material, also known as biofuels, are believed to be less damaging to the environment on combustion, and are obtained from a renewable resource. Certain biofuels may be used as complete substitutes for fuel oils such as diesel fuel oils. Similarly, certain biofuels may be used as partial substitutes for such fuel oils, being blended into the oils in suitable proportions.

Biofuels per se have lower foaming tendencies than typical fuel oils, such as diesel fuel oils. However, it has unfortunately now been found that blends of a biofuel with a diesel fuel oil have much higher foaming tendencies than the fuel oil per se. This finding is surprising since the minor components of fuel oils believed to be responsible for stabilisation of foam and surface-active in nature, differ from the constituents of these biofuels. Consequently, the addition of a quantity of biofuel to a fuel oil was not expected to increase the foaming tendency of the resulting blend.

It has now also surprisingly been found that foaming in a blend of petroleum-based fuel oil and a biofuel may be successfully controlled, in the sense that the initial foam height upon agitation is reduced, by an antifoam additive conventionally used to control foaming in petroleum distillate fuel oils (hereinafter referred to as a petroleum fuel antifoam).

Such additives are themselves surface-active in nature, and are believed to interfere in some way with the foam-stabilising tendency of other components of the fuel blend.

US-A-2 862 885 describes the use of a silicon-containing antifoam for the prevention of foaming of petroleum oil substitutes.

FR-A-2 579 481 describes the use of siloxane-oxyalkylene block copolymers as antifoam agents for hydrocarbon fuel oils.

GB-A-658 494 describes antifoam compositions comprising a water-immiscible organic liquid.

The invention accordingly provides, in a first aspect, a fuel oil composition comprising a major proportion of a blend of petroleum-based middle distillate fuel oil and a biofuel and a minor proportion of a petroleum fuel antifoam, wherein the antifoam is a silicon-containing composition and wherein the fuel oil has a sulphur concentration of 0.05% by weight or less, based on the weight of fuel.

The petroleum fuel antifoams useful in this first aspect of the invention are silicon-containing compositions. It has further been found that foaming in the blend of the first aspect may be successfully controlled, in the sense that foam collapse is accelerated, when the blend contains at most 65% by weight of a biofuel.

The invention accordingly provides, in a preferred embodiment of the first aspect, a fuel oil composition comprising a major proportion of a blend of petroleum-based fuel oil and a biofuel and a minor proportion of a petroleum fuel antifoam being a silicon-containing composition, the fuel oil blend containing at most 65% by weight of a biofuel and at least 35% by weight of a petroleum-based fuel oil.

The invention also provides, in a second aspect, a concentrate comprising a petroleum fuel antifoam in admixture with a blend of a petroleum-based fuel oil and a biofuel; and in a third aspect, the use of a petroleum fuel antifoam to control foaming in a blend of petroleum-based fuel oil and a biofuel.

The invention will hereinafter be described in more detail.

### The Petroleum-Based Fuel Oil (of all aspects of the invention)

The petroleum-based fuel oil is suitably a middle distillate fuel oil, i.e. a fuel oil obtained in refining crude oil as the fraction between the lighter kerosene and jet fuels fraction and the heavier fuel oil fraction. Such distillate fuel oils generally boil within the range of about 100°C to about 500°C (ASTM D-86), e.g. 150°C to about 400°C, for example, those having a relatively high Final Boiling Point of above 360°C, such as 380°C. The fuel oil can comprise atmospheric distillate or vacuum distillate, or cracked gas oil or a blend in any proportion of straight run and thermally and/or catalytically cracked distillates. The most common petroleum distillate fuels are kerosene, jet fuels, diesel fuels, heating oils and heavy fuel oils. The heating oil may be a straight atmospheric distillate, or it may contain minor amounts, e.g. up to 35 wt%, of vacuum gas oil or cracked gas oils or of both. Heating oils may be made of a blend of virgin distillate, e.g. gas oil, naphtha, etc. and cracked distillates, e.g. catalytic cycle stock. A representative specification for a diesel fuel includes a minimum flash point of 38°C and a 90% distillation point of between 282 and 380°C (see ASTM Designations D-396 and D-975).

The fuel oil has a sulphur concentration of 0.05% by weight or less, and preferably 0.01% by weight or less. The art describes methods for reducing the sulphur concentration of hydrocarbon middle distillate fuels, such methods including solvent extraction, sulphuric acid treatment, and hydrodesulphurisation.

### The Biofuel (of all aspects of the invention)

The biofuel may be one or more oils derived from animal or vegetable material or both and capable of being utilised as a fuel.

Oils obtained from animal or vegetable material are mainly metabolites comprising trigylcerides of monocarboxylic acids, e.g. acids containing mainly 10-25 carbon atoms and of the form: where R represents an aliphatic radical of predominantly 10-25 carbon atoms which may be saturated or unsaturated. Preferably, R is an aliphatic radical of 10-25 carbons. Generally, such oils contain glycerides of a number of acids, the number and kind varying with the source of the oil, and may additionally contain phosphoglycerides. Such oils may be obtained by methods known in the art.

Examples of derivatives of such oils are alkyl esters, such as methyl esters, of fatty acids of the vegetable or animal oils. Such esters can be made by transesterification.

Reference within this specification to oils that are derived from animal or vegetable material therefore includes reference both to oils obtained from said animal or vegetable material or both, or to derivatives thereof.

Examples of oils derived from animal or vegetable material are rapeseed oil, coriander oil, soyabean oil, cottonseed oil, sunflower oil, castor oil, olive oil, peanut oil, maize oil, almond oil, palm kemel oil, coconut oil, mustard seed oil, beef tallow and fish oils. Further examples include oils derived from corn, jute, sesame, shea nut, ground nut and linseed and may be derived therefrom by methods known in the art. Rapeseed oil, which is a mixture of fatty acids partially esterified with glycerol, is preferred as it is available in large quantities and can be obtained in a simple way by pressing from rapeseed. Rapeseed oil typically contains the esters of, in addition to some 11 to 19% C₁₆ to C₁₈ saturated acids, some 23 to 32% mono-, 40 to 50% di- and 4 to 12% tri-unsaturated C₁₈ to C₂₂ acids, primarily oleic, linoleic, linolenic and erucic acids.

As lower alkyl esters of fatty acids, consideration may be given to the following, for example as commercial mixtures: the ethyl, propyl, butyl and especially methyl esters of fatty acids with 12 to 22 carbon atoms, for example of lauric acid, myristic acid, palmitic acid, palmitoleic acid, stearic acid, oleic acid, elaidic acid, petroselic acid, ricinoleic acid, elaeostearic acid, linoleic acid, linolenic acid, eicosanoic acid, gadoleic acid, docosanoic acid or erucic acid, which have an iodine number from 50 to 150, especially 90 to 125. Mixtures with particularly advantageous properties are those which contain mainly, i.e. to at least 50 wt% methyl esters of fatty acids with 16 to 22 carbon atoms and 1, 2 or 3 double bonds. The preferred lower alkyl esters of fatty acids are the methyl esters of oleic acid, linoleic acid, linolenic acid and erucic acid.

Commercial mixtures of the stated kind are obtained for example by cleavage and esterification of animal and vegetable fats and oils by their transesterification with lower aliphatic alcohols. For production of lower alkyl esters of fatty acids it is advantageous to start from fats and oils with high iodine number, such as, for example, sunflower oil, rapeseed oil, coriander oil, castor oil, soyabean oil, cottonseed oil, peanut oil or beef tallow. Lower alkyl esters of fatty acids based on a new variety of rapeseed oil are preferred.

Although many of the above oils may be used as biofuels, preferred are vegetable oils or derivatives thereof, of which particularly preferred biofuels are rapeseed oil, cottonseed oil, soyabean oil, sunflower oil, olive oil, palm oil, or alkyl ester derivatives thereof, rapeseed oil methyl ester being especially preferred.

### The Blend (of all aspects of the invention)

The proportion of biofuel in the blend may range from 0.1% to 99.9%, preferably from 0.1% to 90% and more preferably from 0.5% to 85%, by weight. The proportion by biofuel is advantageously at most 65%, and more advantageously at most 55%, by weight.

It is within the scope of the invention to use, as the blend, two or more petroleum-based fuel oils, or more especially two or more biofuels, in admixture with one or more of the other type of fuel.

The blend may contain additives other than the petroleum fuel antifoam. Thus, one or more co-additives such as low temperature flow improvers, stabilisers, dispersants, antioxidants, corrosion inhibitors, cetane improvers, emissions-reducing agents, reodorants, lubricity agents, antistatic additives or demulsifiers may be present in the blend. These co-additives may be added to the blend simultaneously with the petroleum fuel antifoam; for example, the antifoam and co-additives may comprise a single additive. Altematively, one or more co-additives may be added to the blend independent of the antifoam, or to the petroleum-based fuel oil or biofuel prior to blending.

### The Petroleum Fuel Antifoam (of all aspects of the invention)

The antifoam is advantageously insoluble in the fuel being treated but is dispersible therein to form a stable dispersion, if necessary with the aid of a suitable dispersant or solvent, either with or without the use of mechanical dispersing aids.

As the antifoam there may, as indicated above, be used a silicon-containing composition. Such a composition advantageously comprises a siloxane polymer, for example a block copolymer containing siloxane blocks and oxyalkylene blocks. Preferred as such siloxane polymers are those of general formula (i) wherein R represents a hydrocarbyl group, n represents an integer in the range of 1 to 3 and m represents a number ≥ 2. The hydrocarbyl group may be a relatively simple hydrocarbyl group of from 1 to 30 carbon atoms or may be a polymeric group. The groups represented by R may be the same or different in any given siloxane group or throughout the siloxane polymer and the value of n in the various siloxane groups in the siloxane polymer may be the same or different.

The preferred polymers are block co-polymers comprising at least two blocks, one block comprising siloxane groups as represented by general formula (i) and the second block comprising oxyalkylene groups of general formula (ii)

(R¹-O) (ii)

The siloxane block and the oxyalkylene block may be linked to each other by means of a divalent hydrocarbylene group; this may be R in general formula (i). Hence each siloxane block contains at least one group represented by general formula (i) wherein at least one group represented by R is a divalent hydrocarbylene group. The siloxane block has a ratio of hydrocarbyl groups to silicon atoms of 1:1 to 3:1.

The hydrocarbyl groups that are represented by R in general formula (i) may be alkenyl groups for example vinyl and allyl; cycloalkenyl groups, for example cyclohexenyl; alkyl groups, for example methyl, ethyl, isopropyl, octyl and dodecyl; aryl groups, for example phenyl and naphthyl; aralkyl groups, for example benzyl and phenylethyl; alkaryl groups, for example styryl, tolyl and n-hexylphenyl; or cycloalkyl groups, for example cyclohexyl.

The divalent hydrocarbylene groups represented by R in general formula (i) may be alkylene groups such as methylene, ethylene, propylene, butylene, 2,2-di-methyl-1,3-propylene and decylene, arylene groups such as phenylene and p,p'-diphenylene, or alkarylene groups such as phenylethylene. Preferably the divalent hydrocarbylene group is an alkylene group containing from two to four successive carbon atoms.

These divalent hydrocarbylene groups are linked to a silicon atom of the siloxane block by a silicon-to-carbon bond and to an oxygen atom of the oxyalkylene block by a carbon-to-oxygen bond.

The siloxane block in the copolymers may contain siloxane groups that are represented by general formula (i) wherein either the same hydrocarbyl groups are attached to the silicon atoms (e.g. the dimethylsiloxy, diphenylsiloxy and diethylsiloxy groups) or different hydrocarbyl groups are attached to the silicon atoms (e.g. the methylphenylsiloxy, phenylethylmethylsiloxy and ethylvinylsiloxy groups).

The siloxane block in the copolymers may contain one or more types of siloxane group that are represented by general formula (i) provided that at least one group has at least one divalent hydrocarbyl substituent. By way of illustration only, ethylenemethylsiloxy groups can be present in the siloxane block or the siloxane block can contain more than one type of siloxane group, e.g. the block can contain both ethylenemethylsiloxy groups and diphenylsiloxy groups, or the block can contain ethylenemethylsiloxy groups, diphenylsiloxy groups and diethylsiloxy groups.

The siloxane block may contain trifunctional siloxane groups (e.g. monomethylsiloxane groups, CH₃SiO_{1.5}), difunctional siloxane groups (e.g. dimethylsiloxane groups, (CH₃)₂SiO, monofunctional siloxane groups (e.g. trimethylsiloxane groups, (CH₃)₃SiO_{0.5}) or combinations of these types of siloxane groups having the same or different substituents. Due to the functionality of the siloxane groups, the siloxane block may be predominantly linear or cyclic or crosslinked, or it may have combinations of these structures.

The siloxane block may contain organic end-blocking or chain-terminating organic groups in addition to the monofunctional siloxane chain-terminating groups encompassed by general formula (i). Organic end-blocking groups may be hydroxyl groups, aryloxy groups such as phenoxy, alkoxy groups such as methoxy, ethoxy, propoxy and butoxy, and acyloxy groups such as acetoxy.

The siloxane blocks in the copolymers contain at least two siloxane groups that are represented by general formula (i) (so that m represents a number ≥ 2). Preferably, the siloxane blocks contain a total of from five to twenty siloxane groups that are represented by general formula (i), with m representing a number in the range of 5 to 20. That part of the average molecular weight of the copolymer that is attributable to the siloxane blocks may be as high as 50000 but preferably it is from 220 to 20000. If that part of the average molecular weight of the copolymer that is attributable to the siloxane blocks exceeds 50000 or if the siloxane blocks contain a total of more than twenty siloxane groups that are represented by general formula (i), the copolymers are usually not as useful, e.g. they may be too viscous for convenient use in the additives of this invention.

The oxyalkylene blocks in the copolymers each contain at least two oxyalkylene groups that are represented by the general formula (ii) wherein R¹ is an alkylene group. Preferably, at least 60 per cent by weight of such groups represented by general formula (ii) are oxyethylene or oxypropylene groups.

Other oxyalkylene groups that are represented by general formula (ii) which can also be present in the oxyalkylene block, preferably in amounts not exceeding 40 per cent by weight are oxy-1,4-butylene, oxy-1,5-amylene, oxy-2,2-dimethyl-1,3-propylene, or oxy-1,10-decylene groups.

The oxyalkylene blocks in the copolymers may contain oxyethylene or oxypropylene groups alone or along with one or more of the various types of oxyalkylene groups represented by general formula (ii); the oxyalkylene blocks can contain only oxyethylene groups or only oxypropylene groups or both oxyethylene and oxypropylene groups, or other combinations of the various types of oxyalkylene groups represented by general formula (ii).

The oxyalkylene blocks in the copolymers may contain organic end-blocking or chain-terminating groups. Such end-blocking groups may be hydroxy groups, aryloxy groups such as phenoxy, alkoxy groups such as methoxy, ethoxy, propoxy and butoxy, and alkenyloxy groups such as vinyloxy and allyloxy. A single group can serve as an end-blocking group for more than one oxyalkylene block; for example, the glyceroxy group can serve as an end-blocking group for three oxyalkylene chains.

The oxyalkylene blocks in the copolymers contain at least two oxyalkylene groups that are represented by general formula (ii). Preferably, each block contains from four to thirty of such groups. That part of the average molecular weight of the copolymer that is attributable to the oxyalkylene blocks can vary from 176 (for (C₂H₄O)₄) to 200000, but preferably it is from 176 to 15000. Provided that each oxyalkylene block contains at least two oxyalkylene groups represented by general formula (ii), the number of oxyalkylene groups and that part of the average molecular weight of the copolymer that is attributable to the oxyalkylene blocks is not critical, providing that the resulting copolymer is not rendered physically incompatible with oleaginous liquids. However, those copolymers in which that part of the average molecular weight that is attributable to the oxyalkylene blocks exceeds 200000 or that contain more than fifty oxyalkylene groups per block prove less useful, e.g. they are too viscous for convenient use in the additives of this invention.

The copolymers may contain siloxane blocks and oxyalkylene blocks in any relative amounts. In order to possess desirable properties, the copolymer should contain from 5 parts by weight to 95 parts by weight of siloxane blocks and from 5 parts by weight to 95 parts by weight of oxyalkylene blocks per 100 parts by weight of the copolymer. Preferably, the copolymers contain 5 parts by weight to 50 parts by weight of the siloxane blocks and from 50 parts by weight to 95 parts by weight of the oxyalkylene blocks per 100 parts by weight of the copolymer.

The copolymers may contain more than one of each of the blocks and the blocks may be arranged in various configurations such as linear, cyclic or branched configurations.

The most preferred block co-polymers have the general formula (iii) wherein p represents an integer ≥ 2 and preferably represents an integer in the range of 4 to 30, c represents an integer in the range of 0 to 2, m represents an integer ≥ 2, R² represents a monovalent hydrocarbyl radical of 1 to 12 carbon atoms preferably a linear aliphatic radical for example a methyl or ethyl group, R³ represents a divalent hydrocarbyl radical of 1 to 12 carbon atoms preferably an alkylene group of at least two carbon atoms for example ethylene, 1,3-propylene or 1,4-butylene, R⁴ represents the same or different divalent hydrocarbyl radicals of 2 to 10 carbon atoms such as for example ethylene, 1,3-propylene or 1,6-hexylene, and R⁵ represents a monovalent hydrocarbyl group of 1 to 12 carbon atoms or an end-group such as for example hydroxyl or hydrogen. It is preferred that R⁴ represents different hydrocarbyl radicals and most preferably represents a mixture of at least one of each of ethylene and 1,3-propylene radicals.

The above-described block copolymers may be produced by an addition reaction between siloxanes containing silicon-bonded hydrogen atoms and oxyalkylene polymers containing alkenyl end-blocking groups in the presence of a platinum catalyst. These copolymers can also be prepared by a metathesis reaction between siloxanes containing silicon-bonded chloro-organo groups and an alkaline metal salt of a hydroxy end-blocked oxyalkylene polymer.

In accordance with all aspects of the invention, the concentration of the antifoam in the fuel oil composition may for example be in the range of 0.1 to 10,000 ppm, preferably 0.5 to 5000 ppm and most preferably 1 to 100 ppm (active ingredient) by weight per weight of fuel oil. Particularly advantageous concentrations are in the range of 1 to 20 ppm.

### Concentrate

Concentrates are convenient as a means for incorporating the antifoam into the bulk fuel blend. Incorporation may be by methods known in the art. The concentrates may also contain co-additives as required and as hereinbefore described and preferably contain from 3 to 75 wt%, more preferably 3 to 60 wt%, most preferably 10 to 50 wt% of the additives preferably in solution in oil. Examples of carrier liquids are organic solvents including hydrocarbon solvents, for example petroleum fractions such as naphtha, kerosene, diesel and heater oil; aromatic hydrocarbons such as aromatic fractions, e.g. those sold under the 'SOLVESSO' trade name; and paraffinic hydrocarbons such as hexane and pentane and isoparaffins. The carrier liquid must, of course, be selected having regard to its compatibility with the additives and with the fuel blend.

In accordance with the second aspect of the invention, suitable as such a carrier liquid is the fuel blend into the bulk of which the concentrate will be incorporated.

The antifoam may be incorporated into the bulk fuel blend by other methods such as those known in the art. Co-additives may be incorporated into the bulk fuel blend at the same time as the antifoam or at a different time.

The invention will now be illustrated by way of example only as follows:

### Fuels used in the examples

Two petroleum-based fuel oils and a biofuel, having the characteristics shown in Table 1, were used in the following examples of the invention. Both fuel oils were diesel fuels whilst the biofuel was rapeseed methyl ester.

**Table 1**

| Fuel Characteristics | Fuel Oil A | Fuel Oil B | Biofuel |
|---|---|---|---|
| Density, g/ml, 15°C | 0.82 | 0.85 | 0.88 |
| Viscosity, 20°C, mm²/s | 3.09 | 4.7 | 7.22 |
| ASTM-D86 Distillation: (°C) | | | |
| IBP | 168 | 188 | |
| 20% | 203 | 230 | |
| 90% | 330 | 329 | |
| FBP | 371 | 362 | |
| 90-20 | 127 | 90 | |
| 90-FBP | 41 | 33 | |
| Cloud Point, °C (I.S.O. 3015) | -3 ' | -5 | -4 |
| CFPP, °C (E.N. 116) | -5 | -4 | -14 |

### Examples of Antifoams useful in the invention

### (i) Silicon-containing compositions:-

Antifoam A - a proprietary block copolymer comprising siloxane blocks and oxyalkylene blocks, and of the general class hereinbefore described. Antifoam A is sold commercially for the treatment of middle distillate fuel oils.

### Example of the Invention:

The fuel oil compositions defined in Table 5 were prepared by a conventional laboratory blending technique, using a WARING blender. The foaming tendency of each blend of biofuel and petroleum-based fuel oil was measured following addition of antifoam A, using a test procedure involving the agitation by hand of 100 ml of test fuel oil in a previously-cleaned and dried 4 oz bottle, the bottle then being placed in normal attitude on a stationary, flat surface. The subsequent length of time (in seconds) over which the foam generated by shaking collapsed sufficiently to reveal a clear area of liquid surface was recorded as one measure of foaming tendency, longer foam collapse times indicating greater foam stability.

The silicon-containing antifoam significantly reduced foam collapse time in all blends comprising fuel oil A and at most 60% of biofuel (by wt.), and in all blends comprising fuel oil B and at most 70% of biofuel (by wt.) These results suggest the silicon-containing antifoam to be generally effective in fuel oil blends comprising at most about 65% biofuel (by wt.).

The foaming tendency of each blend in Table 5 was also measured in terms of the initial foam height obtained upon agitation. In Table 5, the foam height of each antifoam-containing fuel oil composition is shown (in parentheses) as a percentage of the foam height of the corresponding untreated blend.

The blend foam height results show that initial foam height is generally reduced upon addition of a petroleum fuel antifoam.

## Claims

1. A fuel oil composition comprising a major proportion of a blend of petroleum-based middle distillate fuel oil and a biofuel and a minor proportion of a petroleum fuel antifoam, wherein the antifoam is silicon-containing composition and wherein the fuel oil has a sulphur concentration of 0.05% by weight or less, based on the weight of fuel.

2. A composition as claimed in claim 1, wherein the fuel oil blend contains at most 65% by weight of biofuel and at least 35% by weight of petroleum-based fuel oil.

3. A composition as claimed in claim 2, wherein the blend contains from 0.1% to 65% by weight of biofuel.

4. A composition as claimed in claim 3, wherein the blend contains from 0.5% to 55% by weight of biofuel.

5. A composition as claimed in any one of claims 1 to 4 wherein the fuel oil has a sulphur concentration of 0.01% by weight or less, based on the weight of fuel.

6. A composition as claimed in any one of claims 1 to 5, wherein the middle distillate fuel oil is heating oil or diesel fuel.

7. A composition as claimed in claim 6 wherein the fuel oil is diesel fuel.

8. A composition as claimed in any one of claims 1 to 7, wherein the middle distillate fuel oil has been subject to hydrodesulphurisation.

9. A composition as claimed in any one of claims 1 to 8, wherein the silicon-containing composition comprises a siloxane polymer.

10. A composition as claimed in claim 9 wherein the siloxane polymer is a block copolymer containing siloxane blocks and oxyalkylene blocks.

11. A composition as claimed in claim 9 or claim 10, wherein the siloxane polymer has the general formula (i) wherein R represents a hydrocarbyl or hydrocarbylene group, n represents an integer in the range of 1 to 3 and m represents a number ≥ 2, and wherein the groups represented by R may be the same or different in any given siloxane group throughout the siloxane polymer, and wherein the value of n in the various siloxane groups in the siloxane polymer may be the same or different.

12. A composition as claimed in any one of claims 1 to 11, wherein the biofuel is one or more alkyl esters of fatty acids of vegetable or animal oils.

13. A composition as claimed in claim 12, wherein the alkyl esters are methyl, ethyl, propyl and butyl esters of fatty acids with 12 to 22 carbon atoms.

14. A composition as claimed in claim 12 or claim 13 wherein the alkyl esters are methyl esters of oleic acid, linoleic acid, linolenic acid and erucic acid.

15. A composition as claimed in any one or claims 12 to 14 wherein the biofuel is a mixture containing at least 50 wt % methyl esters of fatty acids with 16 to 22 carbon atoms and 1, 2 or 3 double bonds.

16. A composition as claimed in any one of claims 12 to 15, wherein the biofuel is a rapeseed methyl ester.

17. A composition as claimed in any one of claims 1 to 16, which comprises from 0.1 to 10,000 ppm by weight of antifoam.

18. A composition as claimed in any one of the preceding claims, wherein the blend contains one or more co-additives.

19. A composition as claimed in claim 18, wherein the blend contains, as co-additives, one or more low temperature flow improvers, stabilisers, dispersants, antioxidants, corrosion inhibitors, cetane improvers, emissions-reducing agents, deodorants, lubricity agents, antistatic additives or demulsifiers.

20. A concentrate comprising a petroleum fuel antifoam, wherein the antifoam is a silicon-containing composition, in admixture with a blend of petroleum-based middle distillate fuel oil having a sulphur concentration of 0.05% by weight or less, based on the weight of fuel, and a biofuel.

21. A concentrate as claimed in claim 20 and also containing one or more co-additives.

22. A concentrate as claimed in claim 21, containing one or more co-additives as defined in claim 19.

23. The use of a petroleum fuel antifoam, wherein the antifoam is a silicon-containing composition, to control foaming in a blend of petroleum-based middle distillate fuel oil having a sulphur concentration of 0.05% by weight or less, based on the weight of fuel, and a biofuel.

## Patentansprüche

1. Brennstoffölzusammensetzung, die einen größeren Anteil eines Gemisches aus Mitteldestillatbrennstofföl auf Erdölbasis und Biobrennstoff und einen geringeren Anteil Antischaummittel für Erdölbrennstoff umfaßt, wobei das Antischaummittel eine siliciumhaltige Zusammensetzung ist und das Brennstofföl eine Schwefelkonzentration von 0,05 Gew.% oder weniger hat, bezogen auf das Gewicht des Brennstoffs.

2. Zusammensetzung nach Anspruch 1, bei der das Brennstoffölgemisch höchstens 65 Gew.% Biobrennstoff und mindestens 35 Gew.% Brennstofföl auf Erdölbasis enthält.

3. Zusammensetzung nach Anspruch 2, bei der das Gemisch 0,1 Gew.% bis 65 Gew.% Biobrennstoff enthält.

4. Zusammensetzung nach Anspruch 3, bei der das Gemisch 0,5 Gew.% bis 55 Gew.% Biobrennstoff enthält.

5. Zusammensetzung nach einem der Ansprüche 1 bis 4, bei der das Brennstofföl eine Schwefelkonzentration von 0,01 Gew.% oder weniger hat, bezogen auf das Gewicht des Brennstoffs.

6. Zusammensetzung nach einem der Ansprüche 1 bis 5, bei der das Mitteldestillatbrennstofföl Heizöl oder Dieselkraftstoff ist.

7. Zusammensetzung nach Anspruch 6, bei der der Brennstoff Dieselkraftstoff ist.

8. Zusammensetzung nach einem der Ansprüche 1 bis 7, bei der das Mitteldestillatbrennstofföl Hydrodesulfurierung unterworfen worden ist.

9. Zusammensetzung nach einem der Ansprüche 1 bis 8, bei der die siliciumhaltige Zusammensetzung ein Siloxanpolymer umfaßt.

10. Zusammensetzung nach Anspruch 9, bei der das Siloxanpolymer ein Blockcopolymer ist, das Siloxanblöcke und Oxyalkylenblöcke umfaßt.

11. Zusammensetzung nach Anspruch 9 oder Anspruch 10, bei der das Siloxanpolymer die allgemeine Formel (i) hat, in der R eine einwertige oder zweiwertige Kohlenwasserstoffgruppe bedeutet, n eine Zahl im Bereich von 1 bis 3 bedeutet und m eine Zahl ≥ 2 bedeutet und die von R wiedergegebenen Gruppen in jeder gegebenen Siloxangruppe innerhalb des Siloxanpolymers gleich oder unterschiedlich sein können und der Wert von n in den verschiedenen Siloxangruppen in dem Siloxanpolymer gleich oder unterschiedlich sein kann.

12. Zusammensetzung nach einem der Ansprüche 1 bis 11, bei dem der Biobrennstoff ein oder mehrere Alkylester von Fettsäuren von pflanzlichen oder tierischen Ölen ist.

13. Zusammensetzung nach Anspruch 12, bei der die Alkylester Methyl-, Ethyl-, Propyl- und Butylester von Fettsäuren mit 12 bis 22 Kohlenstoffatomen sind.

14. Zusammensetzung nach Anspruch 12 oder 13, bei der die Alkylester Methylester von Ölsäure, Linolsäure, Linolensäure und Erucasäure sind.

15. Zusammensetzung nach einem der Ansprüche 12 bis 14, bei der der Biobrennstoff eine Mischung ist, die mindestens 50 Gew.% Methylester von Fettsäuren mit 16 bis 22 Kohlenstoffatomen und 1, 2 oder 3 Doppelbindungen enthält.

16. Zusammensetzung nach einem der Ansprüche 12 bis 15, bei der der Biobrennstoff ein Rapssamenmethylester ist.

17. Zusammensetzung nach einem der Ansprüche 1 bis 16, die 0,1 bis 10 000 Gew.ppm Antischaummittel enthält.

18. Zusammensetzung nach einem der vorhergehenden Ansprüche, bei der das Gemisch ein oder mehrere Coadditive enthält.

19. Zusammensetzung nach Anspruch 18, bei der das Gemisch als Coadditive ein oder mehrere Tieftemperatur-Fließverbesserer, Stabilisatoren, Dispergiermittel, Antioxidantien, Korrosionsschutzmittel, Cetanverbesserer (Zündbeschleuniger), Emissionsverminderungsmittel, Deodorantien, Schmierfähigkeitsmittel, Antistatikadditive cder Demulgatoren enthält.

20. Konzentrat, das Antischaummittel für Erdölbrennstoff, wobei das Antischaummittel eine siliciumhaltige Zusammensetzung ist, gemischt mit einem Gemisch aus Mitteldestillatbrennstofföl auf Erdölbasis mit einer Schwefelkonzentration von 0,05 Gew.% oder weniger, bezogen auf das Gewicht des Brennstoffs, und Biobrennstoff umfaßt.

21. Konzentrat nach Anspruch 20, das außerdem ein oder mehrere Coadditive enthält.

22. Konzentrat nach Anspruch 21, das ein oder mehrere Coadditive gemäß der Definition in Anspruch 19 enthält.

23. Verwendung von Antischaummittel für Erdölbrennstoff, wobei das Antischaummittel eine siliciumhaltige Zusammensetzung ist, zur Kontrolle der Schaumbildung in einem Gemisch aus Mitteldestillatbrennstofföl auf Erdölbasis mit einer Schwefelkonzentration von 0,05 Gew.% oder weniger, bezogen auf das Gewicht des Brennstoffs, und Biobrennstoff.

## Revendications

1. Composition de fuel-oil, comprenant une proportion dominante d'un mélange d'un fuel-oil distillé moyen dérivé du pétrole et d'un biocarburant et une petite proportion d'un agent anti-mousse pour carburant dérivé du pétrole, dans laquelle l'agent anti-mousse est une composition contenant du silicium, et le fuel-oil a une concentration en soufre égale ou inférieure à 0,05 % en poids, sur la base du poids du carburant.

2. Composition suivant la revendication 1, dans laquelle le mélange à base de fuel-oil contient au plus 65 % en poids de biocarburant et au moins 35 % en poids de fuel-oil dérivé du pétrole.

3. Composition suivant la revendication 2, dans laquelle le mélange contient 0,1 % à 65 % en poids de biocarburant.

4. Composition suivant la revendication 3, dans laquelle le mélange contient 0,5 % à 55 % en poids de biocarburant.

5. Composition suivant l'une quelconque des revendications 1 à 4, dans laquelle le fuel-oil a une concentration en soufre égale ou inférieure à 0,01 % en poids, sur la base du poids du carburant.

6. Composition suivant l'une quelconque des revendications 1 à 5, dans laquelle le fuel-oil distillé moyen consiste en huile de chauffe ou carburant diesel.

7. Composition suivant la revendication 6, dans laquelle le fuel-oil consiste en carburant diesel.

8. Composition suivant l'une quelconque des revendications 1 à 7, dans laquelle le fuel-oil distillé moyen a été soumis à une hydrodésulfuration.

9. Composition suivant l'une quelconque des revendications 1 à 8, dans laquelle la composition contenant du silicium comprend un polymère de siloxane.

10. Composition suivant la revendication 9, dans laquelle le polymère de siloxane est un copolymère séquencé contenant des séquences siloxane et des séquences oxyalkylène.

11. Composition suivant la revendication 9 ou la revendication 10, dans laquelle le polymère de siloxane répond à la formule générale (i) dans laquelle R représente un groupe hydrocarbyle ou hydrocarbylène, n représente un nombre entier de 1 à 3 et m représente un nombre égal ou supérieur à 2, et les groupes représentés par R peuvent être identiques ou différents dans n'importe quel groupe siloxane donné dans la totalité du polymère de siloxane, et n dans les divers groupes de siloxane dans le polymère de siloxane peut être avoir des valeurs identiques ou différentes.

12. Composition suivant l'une quelconque des revendications 1 à 11, dans laquelle la biocarburant consiste en un ou plusieurs esters alkyliques d'acides gras d'huiles végétales ou animales.

13. Composition suivant la revendication 12, dans laquelle les esters alkyliques sont des esters méthyliques, éthyliques, propyliques et butyliques d'acides gras ayant 12 à 22 atomes de carbone.

14. Composition suivant la revendication 12 ou la revendication 13, dans laquelle les esters alkyliques sont des esters méthyliques d'acide oléique, d'acide linoléique, d'acide linolénique et d'acide érucique.

15. Composition suivant l'une quelconque des revendications 12 à 14, dans laquelle le biocarburant consiste en un mélange contenant au moins 50 % en poids d'esters méthyliques d'acides gras ayant 16 à 22 atomes de carbone, et 1, 2 ou 3 doubles liaisons.

16. Composition suivant l'une quelconque des revendications 12 à 15, dans laquelle le biocarburant est un ester méthylique de colza.

17. Composition suivant l'une quelconque des revendications 1 à 16, qui comprend 0,1 à 10 000 ppm en poids d'agent anti-mousse.

18. Composition suivant l'une quelconque des revendications précédentes, dans laquelle le mélange contient un ou plusieurs co-additifs.

19. Composition suivant la revendication 18, dans laquelle le mélange contient, comme co-additifs, un ou plusieurs agents améliorant l'écoulement à basse température, stabilisants, dispersants, anti-oxydants, inhibiteurs de corrosion, agents améliorant l'indide de cétane, agents diminuant les émissions de polluants, désodorisants, agents d'onctuosité, additifs antistatiques ou désémulsionnants.

20. Concentré comprenant un agent anti-mousse pour carburant dérivé du pétrole, dans lequel l'agent anti-mousse consiste en une composition contenant du silicium, en mélange avec un mélange d'un fuel-oil distillé moyen dérivé du pétrole ayant une concentration en soufre égale ou inférieure à 0,05 % en poids, sur la base du poids du carburant, et d'un biocarburant.

21. Concentré suivant la revendication 20, contenant également un ou plusieurs co-additifs.

22. Concentré suivant la revendication 21, contenant un ou plusieurs co-additifs répondant à la définition suivant la revendication 19.

23. Utilisation d'un agent anti-mousse ou carburant du dérivé du pétrole, dans laquelle l'agent anti-mousse est une composition contenant du silicium, pour s'opposer au moussage dans un mélange d'un fuel-oil distillé moyen dérivé du pétrole ayant une concentration en soufre égale ou inférieure à 0,05 % en poids, sur la base du poids du carburant, et d'un bio-carburant.
